

## 1

3,573,039

## METHOD OF RECOVERING PERSISTENT PHOTOCODUCTORS

Ulo Vahtra and Meredith D. Shattuck, San Jose, Calif., assignors to International Business Machines Corporation, Armonk, N.Y.  
No Drawing. Filed July 18, 1966, Ser. No. 565,687  
Int. Cl. G03g 13/22

U.S. Cl. 96—1

10 Claims

### ABSTRACT OF THE DISCLOSURE

A method of recovering persistent photoconductors is disclosed. After a first image is produced on the photoconductive surface, the surface is uniformly charged to a pre-selected voltage to produce a developable image. The first conductive image is no longer developable.

The invention relates to a photographic reproduction and, more particularly, to a method employing materials which exhibit persistent photoconductivity.

Copending application Ser. No. 474,583, filed July 26, 1965, abandoned in favor of continuation-in-part application, Ser. No. 847,493, filed July 14, 1969, describes a process wherein a persistent photoconductivity member is exposed to a pattern of light to form a latent conductive image in the exposed areas. Next, the exposed surface is brought into contact or near contact with an insulating surface and then separated or peeled away from the insulating surface while a uniform external voltage is applied across the two surfaces. An electrostatic charge pattern corresponding to the conductive pattern of the photoconductor is formed on the insulating surface. This charge pattern on the insulating surface can be developed in any of the conventional ways.

While such a process is highly advantageous for making many copies from one exposure, the persistent photoconductor must be recovered before the photoconductive member can be exposed to a second different image. That is, recovery is defined to mean that the photoconductor can be used to prepare a developed copy of the second image without the first image also being visible on the developed copy.

A further requirement is that the recovery time must be short for the method of Ser. No. 474,583 to be carried out in a reproduction device capable of producing single and multiple copies of the different originals. Normally, recovery of the persistent photoconductor is brought about by heating, which erases or removes the conductive image. The rate of recovery by heat erasure can be increased by increasing the temperature. However, the necessity of increasing the temperature to gain speed or a short recovery time is disadvantageous because many photoconductors show instability when heated, especially repeatedly and in conjunction with exposure to radiation. Thus, the lifetime of the persistent photoconductors becomes limited.

To overcome the shortcomings of heating, other methods of recovery have been conceived. One of these methods has been to expose the persistent photoconductor to infrared radiation, but this technique also appears to work through the generation of heat and has the disadvantages of heat. Moreover, it is less effective than the direct application of heat. Another recovery method is to use direct or alternating electric fields, but with this technique complete recovery of the conductive image is almost never achieved so that the previous images are visible in subsequent copies.

Therefore, it is the primary object of this invention to provide a new and improved recovery method.

## 2

Another object of this invention is to provide a recovery method in which recovery is complete and yet can be achieved at a high rate of speed without shortening the lifetime of the photoconductor.

Still another object of this invention is to provide a recovery method which can be used in conjunction with heat erasures without the heat erasure shortening the lifetime of the photoconductor.

In general, the foregoing and other objects and other advantages are achieved by the following method.

A first conductive image is present in a persistent photoconductor and, by the method of Ser. No. 474,583, one or more copies have been prepared by bringing the surface of the photoconductor into contact with an insulating surface and then separating them, with a unidirectional electrical potential applied across the surfaces, to form, on the insulating surface, an electrostatic image of the conductive image.

Next, to recover the persistent photoconductor in order to prepare a copy of a different image and in accordance with the present invention, the photoconductor is electrostatically charged with the potential applied in the same direction as the potential applied during the step of forming the electrostatic image on the insulating surface and of a magnitude such that the resultant surface potential on the conductive image is greater than  $V - V_{fc}$ , wherein  $V$  is the potential applied during the charge formation on the insulating surface and  $V_{fc}$  is the critical potential at which no charge formation occurs. That is, the polarity of the potential applied to the back of the photoconductor during recovery is the same polarity as the potential applied to the back of the photoconductor during charge formation.

Now, the photoconductor is exposed to a second and different image and, by using the method of Ser. No. 474,583, a copy of the second image is prepared without the first image being visible on the developed copy. However, because the recovery process does not erase the conductive image, both the first and second images may be made visible on the photoconductor by developing it with toner.

The mechanism of the recovery process of the present invention can be explained by an understanding of the charge formation process of Ser. No. 474,583 which is simply defined by the equation:

$$V_f = V_d - V_p + V$$

wherein  $V_d$  is the potential on the insulating surface before charge formation,  $V_p$  is the potential on the surface of the persistent photoconductor before charge formation,  $V$  is the applied potential, and  $V_f$  is the resultant potential of  $V_d$ ,  $V_p$  and  $V$  and is proportional to the potential across the gap between the photoconductive surface and insulation surface. Charge formation will occur when  $V_f$  is greater than  $V_{fc}$ , the critical potential below which charge formation will not occur.  $V_{fc}$  is a function of the width of the gap between the photoconductive surface and the insulating surface, and the gas present in the gap.

Normally,  $V_d$  is assumed to be zero as is  $V_p$  assumed to be zero in the exposed areas of the photoconductor before charge formation.  $V$  is at least 400 volts with the preferred voltage being about 700 volts. Therefore, with the condition that  $V_d$  and  $V_p$  in the exposed areas are assumed to be zero,  $V_f = V$ . In addition, the 400 volts lower limit of  $V$  sets a practical limit on the potential required for charge formation to occur with  $V_d$  and  $V_p$  at zero potential. That is, for this condition,  $V_{fc}$  is established at slightly less than 400 volts for a minimum gap width of less than  $7\mu$  and with air as the gas in the gap. Herein, however, for purposes of description, it will be referenced at 400 volts.

Now, after a persistent photoconductor has been exposed to one image and used in the charge formation process of Ser. No. 474,583 to prepare copies of that image, it must be recovered so that the photoconductor can be exposed to a different image. In accordance with the present invention, the surface of the photoconductor is electrostatically charged with the potential applied to the back of the photoconductor having the same polarity of the potential applied to the back of the photoconductor during the subsequent charge formation and of a magnitude such that the resultant surface potential,  $V_{pe}$ , in the exposed areas of the photoconductor is greater than  $V - V_{fc}$ . The potential  $V$  to be applied during the subsequent charge formation step normally will be the same magnitude as the potential applied during the previous charge formation step.

For purposes of illustrations, a -600 potential is applied to the back of the photoconductor during all charge formation steps and, for purposes of recovery, the surface of the photoconductor is electrostatically charged by a 7000 volt corona unit. That is, a -7000 volt potential is applied to the back of the photoconductor, so that the polarity of both the charge formation potential and the electrostatic charging potential are the same. However, for ease in solving the equation, the back of the photoconductor will be referenced at zero potential and, hence, the charge formation potential or  $V$  is +600 and the electrostatic charging potential is +7000. Accordingly, from the electrostatic charging step or recovery step of the present invention, the previously unexposed areas have a resultant surface potential of about +1000 volts and the previously exposed areas have a resultant surface potential of about +350 volts, depending on the particular photoconductive composition. Turning now to the equation:

$$V_f = V_d - V_p + V$$

wherein  $V_d$  can still be assumed to be zero, but now  $V_p$  in the exposed areas is +350 volts. With  $V$  at +600 volts, it can be seen that:

$$V_f = 0 - (+350) + (+600)$$

$$V_f = +250 \text{ volts}$$

Inasmuch as  $V_{fc}$  is established 400 volts, in this illustration +400 volts,  $V_f$  is less than  $V_{fc}$  and no charge formation will occur. This agrees with the requirement of  $V_{pe} > V - V_{fc}$  for recovery of the exposed areas of the photoconductor. That is, 350 volts is greater than 200 volts (600 volts - 400 volts). Of course, with the unexposed areas having a 1000 volt surface potential, charge formation will not occur in those areas. Now, if the photoconductor is exposed to a different image,  $V_p$  in the newly exposed areas or conductive image again can be assumed to be zero. Thus, in the new conductive areas,  $V_t = V$ , and hence  $V_f$  will be +600 volts which is greater than  $V_{fc}$  (+400 volts) and charge formation will occur. Thus, developed copies of the different image can be prepared on insulating surfaces by the process of Ser. No. 474,583 without the first conductive image also being developed.

Any photoconductor capable of forming a latent conductivity image on exposure can be used in the process of the present invention. This includes photoconductors, such as those described in copending application Ser. No. 474,977 filed July 26, 1965 now U.S. Pat. 3,512,966, which can be recovered by one of the above known methods and also photoconductors, such as those described in U.S. Pat. 3,113,022, which cannot be recovered by one of the above known techniques, i.e.—heat. Of course, photoconductors, such as selenium, whose conductivity does not remain or persist after the exposing light is removed and, hence, are not useful in the method of Ser. No. 474,583 or, in other words, the process of the present invention is not applicable to non-persistent photoconductors.

Turning now to a discussion of the method of Ser. No. 474,583 in a conventional electrophotographic machine environment with the photoconductor carried on a drum to show how the recovery method of the present invention improves the method of Ser. No. 474,583 so that it can be employed as a high speed reproduction method. In the method of Ser. No. 474,583, a previously unexposed persistent photoconductor is exposed to a pattern of light and dark from a first original or master to form a conductive image in the photoconductor. Next, the exposed surface of the photoconductor is brought into contact with the insulating surface of a dielectric sheet and, at least during the separation of the photoconductor from the dielectric sheet, a potential is applied across them, which is sufficient in magnitude to form an electrostatic charge pattern on the insulating surface corresponding to the conductive image. Preferably, an electrostatic charge is applied to the surface of the photoconductor prior to the application of the potential across the photoconductor and dielectric sheet and of such a polarity to prevent electrostatic charge formation on the insulating surface of the dielectric sheet corresponding to the non-conductive or insulating areas of the photoconductor. This step is only necessary before the first charge formation copy because the charge will be retained on the non-conductive or insulating areas of the photoconductor during the formation of subsequent charge patterns on dielectric sheets of the same conductive image.

Of the above steps in the method of Ser. No. 474,583, it primarily is the exposure step which limits the speed of operation in making one copy of the first original. This is because the charge formation step and the preferred charging step can be carried out at a higher rate of speed than the exposure step of the photoconductor due to the light sensitivity of the photoconductor. Generally speaking, the photoconductor can travel at a speed of about at least 200 linear feet per minute for the charge formation and charging steps whereas, depending on the particular photoconductor, can only travel at a speed of about 20 linear feet per minute if the exposure step is optical and about 100 linear feet per minute if contact exposure is used. However, only one exposure is needed for multiple copies of the same original so that, overall, the machine employing the method of Ser. No. 474,583 can operate as a high speed reproduction device if only multiple copies of the same original is desired.

On the other hand, if the machine is to produce copies of different originals by contact exposure using the method of Ser. No. 474,583, the speed of operation is primarily dependent upon the heat recovery or erasure time of the photoconductor because the photoconductor can only travel at about a speed of about 60 linear feet per minute for 150° C. heat erasure step. However, if in place of the heating step of Ser. No. 474,583 the recovery method of the present invention is used, the limiting step on the speed of operation again is the exposure step in exposing of the second original. That is, the recovery method of the present invention only requires an electrostatic charging step which can be carried out at about at least 200 linear feet per minute, a faster rate of speed than the exposure speed of the photoconductor.

Now, the photoconductor can be exposed to a pattern of light and dark from a second and different original and the charge formation method of Ser. No. 474,583 can be employed to make one or multiple copies of the second original. Again, no additional exposure step is necessary for the multiple copies. Therefore, it should be apparent that the present invention makes the method of Ser. No. 474,583 practical for use in a reproduction device preparing not only multiple copies of one original but single and multiple copies of many different originals at a high rate of speed.

It will be remembered that the first conductive image was not erased by the recovery method of the present invention because if the photoconductor is developed by

a conventional technique, such as cascade development, both the first and second conductive images are visible. These conductive images are not permanent, except for possibility the materials of U.S. Pat. 3,113,022, and persist from minutes to days depending upon the particular composition of the photoconductor. Therefore, the conductive images will gradually become erased at room temperature over a period of time. If desired, however, heat erasure can be used in conjunction with the process of the present invention and can be employed infrequently so as not to shorten the lifetime of the photoconductor. For example, the heating means of Ser. No. 474,583 could be included in a high speed reproduction device and operated only when the reproduction device was being shut off, such as the end of the day. In this way, the conductive images would be erased without affecting the high speed operation of the reproduction device or shortening the lifetime of the photoconductor.

The general nature of the invention having been set forth, it now will be further illustrated by reference to the following specific examples in which the criticalness of the polarity of the potential applied to the photoconductor for recovery of the conductive image will be shown. In addition, the following examples will show that the recovery process of the present invention is operable on both reversible and irreversible persistent photoconductive materials.

In these examples, the terms "negative" or "positive," when they relate to electrostatic charge patterns or toner, connote the polarity of the charge of the pattern or the toner. On the other hand, when these terms are applied to a master, they are definitive as to whether the information or background is dark. That is, this patent is a positive master because the print, not the background, is dark. On the other hand, if the master is a transparency in which the print areas are transparent and the background dark, this would be a negative master. This same definition is true when the terms positive and negative are applied to copies. A different master is a master that would interfere and overlap the image areas of a previous master. Of course, the photoconductor can be re-exposed to the same master. In this case, the recovery step is employed so that accurate alignment of the two exposures and, hence, conductive images is not necessary to prevent the copies from being blurred.

#### EXAMPLE I

A persistent photoconductive film was prepared by dissolving 10 mg. of Malachite Green oxalate and 40 mg. 3,5-dinitrobenzoic acid in a small amount of methanol to which was added 14.3 g. of a solution of 5.3% of polyvinylcarbazole in dichloroethane. This solution was coated on an aluminum foil using a 5 mil wet gap. The prepared film was exposed to a 40 watt incandescent lamp at 12 inches through a negative master for two seconds. The film then was run several times through a charge formation station, each time being sandwiched with a dielectric paper having an insulating surface. The charge formation station was maintained at 600 volts with the positive polarity being applied to the back of the photoconductor. Positive electrostatic charge impressions corresponding to the exposed areas of the photoconductive film were formed on each dielectric paper and were made visible with commercially available positive going (negative) toner particles applied with a magnetic brush to form positive copies of the negative master.

To recover the photoconductive film for a different image, the photoconductive film was electrostatically charged with a corona unit at a 7000 volt potential. That is, a positive 7000 volts was applied to the back of the photoconductive film and, thus, was the same polarity as was applied to the photoconductor back during the charge formation step. Next, the photoconductive film was exposed to a 40 watt incandescent lamp at 12 inches through a different negative master for two seconds.

After carrying out the same charge formation step and development step, the dielectric paper was observed to see if the prior conductive image had been formed and developed. The prior image from the first negative master was not visible. The above process was repeated several times, each time exposing the photoconductive film to a different image. In each case, the prior image(s) did not appear on the developed dielectric paper, but only a good quality positive copy of the negative image, from the exposure after the electrostatic charging step or recovery step, was produced.

#### EXAMPLE II

Using the photoconductive film of Example I and the procedural steps of recovery, exposure of a first positive master, charge formation, recovery, exposure of a second and different positive master, and charge formation, positive copies were prepared of the second positive master. The polarity of the potential applied to the back of the photoconductor during both the charge formation step and the electrostatic charging step for recovery was reversed from that of Example I so that negative polarity was applied to the back of the photoconductive film. The electrostatic charge impressions on the dielectric papers were developed by cascade development with a commercially available positive going (negative) toner. Good quality positive copies of the second positive master were obtained without the images from the first positive master being visible.

#### EXAMPLE III

Using the photoconductive film and procedure steps of Example I, the photoconductive film was exposed to 20 different images and from one to twenty electrostatic impressions were formed on dielectric papers from each image. In each case, the previous image(s) was not visibly present on the subsequent dielectric copy. That is, only a good quality copy(ies) of the image after recovery was developed.

#### EXAMPLE IV

In support of the mathematical explanation previously given, the photoconductive film of Example I was exposed uniformly to a 40 watt incandescent lamp at 12 inches for two seconds. Using the charge formation technique of Example I, six electrostatic charge impressions were made on six dielectric papers using a 600 volt potential of the same polarity as Example I. Next, the completely exposed photoconductive film was measured with an electrometer and found to have a surface potential of +20 volts. The same procedure then was carried out with an unexposed film which, when measured with the electrometer, had a surface potential of +105 volts after six charge formations. However, when these films were electrostatically charged with a corona unit at 6000 volts potential and in the same direction as the charge formation potential, the surface potential of the exposed film was +350 volts and the surface potential of the unexposed film was +1000 volts.

#### EXAMPLE V

Using the film formulation of Example I, a previously unexposed photoconductive film was exposed through a target to a 40 watt incandescent lamp at 12 inches for two seconds. According to the recovery process of the present invention, the film then was charged with a corona unit set at 6500 volts with the positive polarity applied to the back of the photoconductor. Next, instead of carrying out a charge formation step with a dielectric paper, the film was given a short uniform exposure to dissipate the electrostatic charge and, after this, the charge formation step was performed and a positive electrostatic charge pattern of the exposure image formed on a dielectric paper which was developed. Thus, this example shows that, without a surface potential greater than  $V - V_{fc}$  in the previously exposed areas being present, a charge

formation image will still result. Also, the example shows that the electrostatic charging step for recovery does not erase a conductive image.

#### EXAMPLE VI

For further understanding of the recovery process of the present invention, a previously unexposed photoconductive film of the formulation of Example I was exposed through a positive master to a 40 watt incandescent lamp at 12 inches for two seconds. The photoconductor then was charged by a corona unit at 6500 volts with the positive polarity applied to the back of the photoconductor. Next, using the charge formation technique of Example I, except that the polarity of the potential was reversed and the negative polarity supplied to the back of the photoconductor, the photoconductor in contact with a dielectric sheet was passed through the charge formation station. That is, the polarity applied to the back of the photoconductor by the corona unit and the charge formation unit was opposite rather than the same, which is required by the recovery process of the present invention. With this reverse polarity, an electrostatic image was formed and developed on the dielectric paper whereas if the polarity had been the same as in Example I, no image would have formed.

#### EXAMPLE VII

To show that the above results occur with a negative master as well as a positive master, the procedure of Example VI was followed, except that a negative master was used and the polarity of the potential of the corona unit applied to the back of the photoconductor was negative and the polarity of the charge formation potential applied to the back of the photoconductor was positive. Again, the exposed image was not recovered and an electrostatic image was formed and developed on the dielectric paper.

#### EXAMPLE VIII

A photoconductive coating was prepared according to U.S. Pat. 3,113,022, in which the conductive images are essentially irreversible or not erasable by known techniques. That is, a diazonium salt, 0.02 gram of 2,5-dimethoxy - 4 - benzoylaminobenzene diazonium fluoroboride, was dissolved in 2 ml. of acetonitrile and the solution added to 10 percent solution of polymethylmethacrylate in 2-butanone. The resulting solution was coated on aluminum foil with a 5 mil wet gap. The coating then was cured at 60° C. Using the procedural steps of Example I, the coating was exposed through a negative master to a 500 watt photoflood lamp at 12 inches for sixty seconds. Next, the film was contacted to a dielectric paper and passed through a pair of conductive rollers at a potential of 600 volts and with the positive polarity being applied to the back of the photoconductor. The charge formation step was repeated three times to give three electrostatic charge impressions on three dielectric papers, which were developed and yield good quality copies of the master. To recover the photoconductive film, the film then was charged with a corona unit at 7000 volts with the positive polarity being applied to the back of the photoconductor. Now, the photoconductor was exposed to a second and different master and, by repeating the charge formation step above, an electrostatic charge impression corresponding to the image of the second master was formed on the dielectric paper. After developing the electrostatic charge impression, the paper was examined and a good quality copy of the second image was present without the first exposure image being visible. Two more copies of different masters were prepared using this recovery process. In each copy, the previous image was not visible.

#### EXAMPLE IX

After the three different copies from three different exposure images were prepared by the charge formation

technique in Example VIII, the photoconductor was again electrostatically charged to the same potential and the same polarity and the photoconductor was cascade developed with a commercially available negative going (positive) toner. All three different images to which the film was exposed in Example VIII were developed and visible.

#### EXAMPLE X

A photoconductive composition of a solution of 30 mg. of 2,2',4,4',6,6'-hexanitrodiphenylamine, 5 mg. of Malachite Green oxalate and 0.5 g. of 1,3-diphenyl-5-(4-dimethylaminophenyl)-pyrazoline in 5 ml. of 1,2-dichloroethane was added to a solution of 2 g. of polystyrene in 18 g. of benzene. The resulting solution was coated on an aluminum foil with a 7 mil wet gap. The film then was exposed through a negative master to a 40 watt incandescent lamp at 12 inches for two seconds. Next, the film was passed through conductive rollers at 900 volts potential to show that the recovery process of the present invention is operable with electrostatic charging means other than a corona unit. The positive roller or polarity was applied to the conductive aluminum backing of the film. Next, the film was re-exposed to a second and different master and several charge formations made with dielectric papers at 600 volts potential, with the negative polarity being applied to the back of the photoconductor as was the case in the previous recovery step. The dielectric papers were developed in the same manner as Example I. In each case, the previous image was not visible on the developed dielectric paper.

#### EXAMPLE XI

To show that the recovery process of the present invention is operable with inorganic persistent photoconductors, a solution of 7.5 g. of polymethylmethacrylate in 40 g. of toluene was added 0.006 g. of Rhodamine B in 3.5 g. of methanol and 22.5 g. of electronic grade zinc oxide. The mixture was dispersed by a high speed stirrer and coated on an aluminum foil with a 3 mil wet gap. The thus prepared photoconductive film was exposed through a first negative master for 10 seconds to a 40 watt incandescent lamp at 12 inches. Next, the photoconductor was contacted with a dielectric paper and passed through a pair of conductive rollers at a potential of 600 volts and with the positive polarity being applied to the back of the photoconductor. The electrostatic charge pattern which formed on the dielectric paper was developed to yield a good quality copy. To recover the photoconductor, a 6000 volt potential from a corona unit was applied to the photoconductor, with the positive polarity being at the back of the photoconductor. The recovered photoconductor then was exposed to a second and different negative master with the same lamp, distance, and time as described above. Repeating the charge formation and development procedure used for the copy of the first master, a good quality copy of the image of the second master was produced without the first image being visible. Finally, a good quality copy of a third and different master was prepared without the first and second images being visible by the above described steps of electrostatically charging the photoconductor, exposing it through the third master, forming a charge impression on a dielectric paper and developing the charge impression.

While the invention has been particularly shown and described with reference to preferred embodiments thereof, it will be understood by those skilled in the art that variations in form may be made therein without departing from the spirit and scope of the invention.

What is claimed is:

1. In the process of forming a developable electrostatic charge pattern on a member having an insulating surface by applying a unidirectional electric field across said member and the surface of a persistent or essentially irreversible photoconductive element contiguous with the

surface of said member and having a first conductive image, the step of recovering the photoconductive element comprising:

5 electrostatically charging the photoconductor while it still contains said conductive image with the applied potential being in the same direction as the potential applied during the step of forming the electrostatic charge pattern on the insulating surface and of a magnitude such that the resultant surface potential on the conductive image is greater than  $V - V_{fc}$ , wherein V is the potential of said electric field applied during the formation of the electrostatic charge pattern on the insulating surface and  $V_{fc}$  is the critical potential at which no charge formation will occur, whereby a second conductive image can be induced in the photoconductor and a developable electrostatic charge pattern corresponding to said second conductive image can be formed on an insulating surface without a developable electrostatic charge pattern corresponding to the first conductive image also being formed.

2. The process of claim 1 wherein said second conductive image is different from said first conductive image.

3. The process of claim 1 wherein  $V_{fc}$  is about 400 volts.

4. The process of claim 3 wherein V ranges from above about 400 volts to about 900 volts.

5. The process of claim 1 wherein the conductive image formed in said photoconductor is essentially irreversible.

6. A reproduction process for producing copies of at least two originals comprising the steps of:

(a) exposing a photoconductive member capable of exhibiting persistent or essentially irreversible photoconductivity to a pattern of light and dark from a first original to induce electrical conductivity in the light exposed areas;

(b) placing a member having an insulating surface in contact with the exposed surface of the photoconductive member;

(c) separating said members with a uniform electric field applied across the surfaces whereby an electrostatic charge pattern is formed on the insulating surface corresponding to said pattern of light and dark;

(d) developing the electrostatic charge pattern to render it visible;

(e) electrostatically charging the photoconductive

member while it contains a conductive image with the applied potential being in the same direction as the potential applied during the step of forming the electrostatic charge pattern on the insulating surface and of a magnitude such that the resultant surface potential on the conductive image is greater than  $V - V_{fc}$ , wherein V is the potential of said electric field applied during the formation of the charge pattern on the insulating surface and  $V_{fc}$  is the critical potential at which no charge formation will occur;

(f) exposing said photoconductive member to a pattern of light and dark from a second original to induce electrical conductivity in the light exposed areas; and

(g) repeating the steps b, c, and d whereby an electrostatic charge pattern of only the pattern of light and dark from the second original is formed and developed on an insulating surface.

7. The process of claim 6 wherein said second original is different from said first original.

8. The process of claim 6 wherein  $V_f$  is about 400 volts.

9. The process of claim 7 wherein V ranges from above about 400 volts to about 900 volts.

10. The process of claim 6 wherein the conductive image formed in said photoconductor is essentially irreversible.

#### References Cited

#### UNITED STATES PATENTS

|           |         |                |       |          |
|-----------|---------|----------------|-------|----------|
| 2,833,648 | 5/1958  | Walkup         | ----- | 96—1     |
| 2,857,290 | 10/1958 | Bolton         | ----- | 117—17.5 |
| 2,982,647 | 5/1961  | Carlson et al. | ----- | 96—1     |
| 3,005,707 | 10/1961 | Kallman et al. | ----- | 96—1     |
| 3,013,878 | 12/1961 | Dessauer       | ----- | 96—1     |
| 3,041,167 | 6/1962  | Blakney et al. | ----- | 96—1     |
| 3,084,061 | 4/1963  | Hall           | ----- | 117—17.5 |
| 3,147,679 | 9/1964  | Schaffert      | ----- | 95—1.7   |
| 3,268,331 | 8/1966  | Harper         | ----- | 96—1     |
| 3,322,538 | 5/1967  | Redington      | ----- | 96—1.1   |
| 3,355,289 | 11/1967 | Hall et al.    | ----- | 96—1.4   |

GEORGE F. LESMES, Primary Examiner

45 J. C. COOPER III, Assistant Examiner

U.S. Cl. X.R.

96—1.3, 1.4; 117—17.5